

# UNITED STATES PATENT OFFICE.

ISAIAH L. ROBERTS, OF LOCKPORT, NEW YORK.

## PROCESS OF MAKING ACID OR ALKALI RESISTING ARTICLES.

992,256.

Specification of Letters Patent. Patented May 16, 1911.

No Drawing.

Application filed July 23, 1907. Serial No. 385,215. (Specimens.)

To all whom it may concern:

Be it known that I, ISAIAH L. ROBERTS, a citizen of the United States, residing at Lockport, in the county of Niagara and State of New York, have invented certain new and useful Improvements in Processes for Making Acid or Alkali Resisting Articles, of which the following is a specification.

My invention relates to articles of wood, 10 wood-pulp, straw-board or other woody material, to be used with acids or alkalies or both, and has for its object to provide an article for such purpose which shall be capable of resisting the attacks of acids and alkalies, and to provide an economical and 15 easily practiced process or method for making such articles.

Heretofore numerous attempts have been made to utilize wood, wood-pulp, etc., for 20 articles to be used with acids and alkalies, for example, as containing receptacles or vessels for the same, but so far as I am aware none of these attempts has been wholly successful. A common method for the purpose 25 is to coat the surface of the article, or to impregnate the article as deeply as possible, with acid and alkali resisting material; but it has been found that after an article so treated has been in use for a more or less 30 short time the chemical, especially if it be an acid, attacks the ends of the fibers at the contact surface, and following these fibers soon permeates the article and greatly impairs it or renders it entirely useless.

25 In carrying out my present invention in the preferred manner I make the desired article, for instance a vessel, by turning the same from a block of wood in a lathe, or fashion it of wood-pulp, papier-mâché, 40 strawboard, or similar material, in any convenient way. The article is then partially "carbonized," in the manner described in my prior application Ser. No. 253,384, filed April 3, 1905, patented October 5th, 1909, No. 45 936,039. To effect the partial carbonization the article is placed in an oven and heat applied, very slowly and evenly so that the article will not be cracked by sudden change of temperature. As the carbonization pro-

ceeds the article shrinks more or less, but if the heating is gradual no splitting or cracking will occur. The extent to which the heating should be carried, depends in general upon the material of which the article 50 is made, and the size thereof or the thickness of its walls, and for particular mate-

rials and conditions can best be determined by trial. In general it may be stated that the carbonization should proceed throughout the entire body of material and until the 60 article is porous, resembling charcoal in appearance, but must leave the article strong enough to serve its intended purpose. The cooling must also be slow and even, like the heating, to avoid the cracking which might 65 be caused by sudden change of temperature. The partially carbonized article is now treated, as for example by soaking or boiling, with an alkali or acid resisting substance or substances to render it impervious 70 thereto. For this purpose the article may be immersed in liquefied wax, such as paraffin, beeswax, ozokerite, etc.; or liquefied tar, resin, asphaltum, etc., sulfur, or even stearic acid; until the pores of the article are permeated with the resistant material. If desired, a mixture of two or more of the above substances may be used. For instance, asphaltum is more or less viscous when melted, so much so as to be absorbed into the pores 80 slowly; in this case resin and paraffin may be mixed with the asphaltum in sufficient quantities to give the desired fluidity.

What particular substance or substances are to be used will depend somewhat upon 85 the cost and weight thereof, but primarily upon the particular use for which the article is intended. For example, stearic acid and hydrocarbon waxes will resist practically all acids, but the paraffin waxes, or sulfur, 90 should be used if resistance to alkalies is desired.

When the article is well permeated the permeating material is allowed to harden, whereupon the article is ready for use. Such 95 an article is completely impervious and resistant, resisting admirably even slow attack on the surface fibers, and hence has very long life with strong acids or alkalies.

The resistant substances hereinbefore 100 named are the most suitable for the purpose and a number of them are very inexpensive; at the same time they are not heavy enough to make the article inconveniently heavy. In general any impervious resistant substance or mixture of substances can be used which can be liquefied, as by heat, or in a solvent, etc., and which will harden again in the pores of the article.

105 What I claim is:

110 1. The method of treating articles of woody material to make the same liquid-

proof and acid or alkali resistant, which consists in partially carbonizing the article throughout the body of material, and then filling the pores thereof with resistant material.

2. The method of treating articles of woody material to make the same liquid-proof and acid or alkali resistant, which consists in partially carbonizing the article throughout the body of material, then filling the pores thereof with resistant material liquefied by heat, and allowing the material to harden in the pores of the article.

3. The method of treating articles of woody material to make the same liquid-<sup>15</sup> proof and acid or alkali resistant, which consists in gradually heating the article until partially carbonized through the body of material, and then filling the pores of the partially carbonized article with resistant <sup>20</sup> material.

ISAIAH L. ROBERTS.

Witnesses:

WM. H. BAKER,  
M. J. NELLIGAN.